

Oct. 25, 1927.

1,646,667

J. M. TOBIN

METHOD OF MAKING FLOORS

Filed March 1, 1922



INVENTOR  
John M. Tobin

BY  
David Rines  
ATTORNEY

## UNITED STATES PATENT OFFICE.

JOHN MICHAEL TOBIN, OF SOMERVILLE, MASSACHUSETTS, ASSIGNOR TO WILLIAM M. BAILEY COMPANY, OF BOSTON, MASSACHUSETTS, A CORPORATION OF MASSACHUSETTS.

## METHOD OF MAKING FLOORS.

Application filed March 1, 1922. Serial No. 540,101.

The present invention relates to methods of making floors and the like, more particularly concrete or terrazzo-like floors.

The object of the invention is to provide 5 a concrete or terrazzo-like floor or similar surface that shall have as nearly as possible the hardness of the constituent stone employed in its manufacture.

The single figure of the drawing is a 10 view, in cross section, of a bottom upon which the floor is to be laid, with the constituent materials laid thereon, before the materials have been compacted and the floor finished.

15 As a preliminary operation, the surface 2 of the old concrete is treated with picks or the like until the solid aggregate is exposed. It is then thoroughly cleaned of all loose concrete, dust, dirt and other particles, after 20 which it is washed. It is essential that these fine particles be removed before the washing, for it is not possible to remove them when wet. The excess water is swept away with stiff bristle brooms, leaving the 25 surface 2 as nearly clean as it is possible to have it.

A grout 4 of cement and water is then 30 poured over the surface 2, and the surface 2 is thoroughly treated with the same, as by means of stiff brushes, so that all portions of the surface shall become intimately coated with the cement. This will facilitate the bonding to the surface 2 of the layer 6 of cement and stone placed thereover.

35 This layer comprises different-sized stones, such as trap rock, and cement mixed together, in suitable proportions. The stones should be of the same character throughout in order that the final floor may be homogeneous. Stones of two average sizes have 40 been found to work well in practice. The larger stones may be of a size adapted to pass through a  $\frac{3}{4}$  inch ring and to be retained upon a  $\frac{3}{8}$  inch ring. The smaller 45 stones may be of a size that will pass through a  $\frac{3}{8}$  inch ring and that will be retained upon a  $\frac{1}{8}$  inch ring. Stones of these sizes, in the proportion say, of one volume of the small size to three volumes of the large size, 50 may then be mixed with half their aggregate volume of cement. The mixture is preferably of a consistency such that, when dumped from a wagon, it will form into an up-standing mass. This mass is then

brought to the level of previously positioned 55 screeds in a manner well known.

The above-given sizes and proportions have been found to yield very satisfactory results for indoor flooring an inch or so in thickness. The sizes and the proportions 60 may be varied to suit the needs of the particular job in hand. For thicker floorings, for example, stones of much larger size may be employed; and it is not essential that two sizes only may be employed, the essential 65 requirement being that the sizes and the proportions be such that in the finished floor, the smaller stones will fill the interstices between the larger stones as completely as 70 possible, thereby approximating, as nearly as may be, to a solid stone floor. The stones should not, however, be of two small a size, say the size of sand grains, for the subsequent operations will force such smaller particles to the surface, producing a "dusty" 75 floor and one of less hardness and durability.

After the screeds are removed, a further layer 8 is superposed over the layer 6. The layer 8 consists of the same stones as are 80 used in the layer 6, and in about the same proportions; but without the cement. It is scattered or sprinkled over the layer 6 from pails carried by the workmen to a depth such that the final proportion of cement to 85 stone is about one to three. This layer 8 is trowelled into the layer 6 in any well known way, as by means of a steel trowel and wood floats. This operation lasts for 90 an hour, more or less, according to circumstances.

The mass is then compacted until the stones are forced into a position approximating as closely as possible to a layer of solid rock, the smaller stones filling up, as 95 nearly as may be, the interstices between the larger stones; and the remaining space being filled by the cement. A good deal of the cement is forced to the surface by the compacting process, and is removed, so that 100 the volume of voids between the stones that is occupied by the cement in the completed floor is estimated to be not more than ten to fifteen per cent.

The most satisfactory method now known 105 for compacting the mass is to roll it. Rolling flooring of the type described is not, of course, new; but such rolling hitherto has been for

the purpose of leveling it off rather than to compact the constituent stones. If a heavy enough roller were employed, in fact, with this end in view, the roller would sink into the mass and drive the aggregate out of shape, defeating the purpose for which it is intended.

According to the present invention, however, comparatively light rollers are used at first. The rollers are moved across the floor both lengthwise and crosswise of the floor for a period of time sufficient to cause the individual stones to assume positions such that a heavier roller may then be employed without dislodging them. For the making of a floor of the above described character, the initial rolling may be effected with rollers two feet wide weighing about one hundred pounds.

20 The rollers next employed may be twice as heavy, and their purpose is further to compact the mass. After these have been employed for a sufficient length of time, depending upon circumstances, they are replaced by rollers weighing about twice as much, but whose weight is distributed over a greater length. Three rollings of this character are usually sufficient, in practice. In this manner, it is possible to employ rollers during the second and third rollings that it would not be possible to use at all in the beginning, and to compact the stones together in a way that hitherto has been thought to be impossible. The final rolling, 35 of course, should be effected before the mass has obtained its initial set.

As the stones are forced by the successive rollings closer and closer to the final positions, the interstices between them become 40 smaller and smaller, so that excess cement, water, laitance, and other foreign materials are gradually forced to the surface and out of the mass. If sand or fine particles of stone were employed, these would also be forced to the surface, and as they could not, probably, be wholly removed in this manner, they would continue to come to the surface during subsequent heavy use of the floor, causing a "dusty" surface. This 45 furthermore, would render the surface of the floor less hard. It is for this reason, furthermore, that the mixture of stone and cement that forms the layer 6 is made as dry as possible. The introduction of excess water would simply delay the work, as it would have to be squeezed out by the rollings.

The ridges caused by the rollers are smoothed out by steel trowels, and the floor, 60 thus finally leveled, is allowed to set. It is flooded with water to a suitable depth after some fourteen hours' wait, depending upon the temperature and other factors, and it is maintained flooded for a suitable number 65 of days. The hardened scum, laitance, etc.,

is finally ground away, and the floor is allowed to dry, after which it is ready for use.

It has heretofore been proposed to roll surfaces with rollers of successively increasing weight. According to the present invention, however, the constituent stones are first so selected and graded that, after they have been compacted together by such successive rollings, the smaller size stones substantially fill the interstices between the larger-size stones, the resulting floor being terrazzo-like in appearance, but seeming to have all the attributes of solid rock. Besides being hard and wear-resisting, these floors are absolutely dustless. Floors constructed in this manner have shown no appreciable signs of wear, though subjected to the hardest sort of usage over a period of years.

The term "floor" has been employed above, and will be employed in the claims, to signify not merely indoor traffic surfaces, but also other surfaces, such as sidewalks and the like that are required to be of an intensively resistant character.

It will be understood that the invention is not restricted to the exact embodiment that has been illustrated and described herein. Changes may be made by persons skilled in the art, but such changes are considered to be within the spirit and scope of the invention, as defined in the appended claims.

What is claimed as new is:

1. The method of making a terrazzo-like floor that comprises placing upon a suitable bottom a layer of stones of substantially different sizes mixed with cement, and rolling the layer during suitable successive periods of time with rollers of successively increasing weight.

2. The method of making a terrazzo-like floor that comprises mixing with cement stones of substantially different sizes of dimensions and in volumes such that the smaller-size stone shall substantially fill the interstices between the larger-size stones, placing a layer of the mixture upon a suitable bottom, and rolling the layer during suitable successive periods of time with rollers of successively increasing weight.

3. The method of making a terrazzo-like floor that comprises mixing, with half their aggregate volume of cement, stones of substantially two sizes, in the proportion of substantially one volume of the smaller stones to substantially three volumes of the larger stones, the average size of the smaller stones being substantially half the average size of the larger stones, placing a layer of the mixture upon a suitable bottom, and rolling the layer during suitable successive periods of time with rollers of successively increasing weight.

4. The method of making a terrazzo-like floor that comprises mixing with cement stones of substantially different sizes and of

dimensions and in volumes such that when the stones are compacted together the smaller-size stones shall substantially fill the interstices between the larger-size stones, the 5 stones having about the hardness of trap rock, placing a layer of the mixture upon a suitable bottom, and compacting the mass together by acting upon its surface during suitable successive periods of time with tools 10 adapted to exert during the successive periods successively increasing compacting forces to force the excess laitance and other foreign matter out of the mass and to cause the smaller-size stones substantially to fill the interstices between the larger-size stones, 15 whereby the resulting floor will be of about the hardness of a solid trap-rock surface.

5. The method of making a terrazzo-like floor that comprises mixing with cement 20 stones of substantially different sizes and of

dimensions and in volumes such that when the stones are compacted together, the smaller-size stones shall substantially fill the interstices between the larger-size stones, the stones having about the hardness of trap 25 rock, placing a layer of the mixture upon a suitable bottom, and compacting the mass together by rolling it during suitable successive periods of time with rollers of successively increasing weight to force the excess laitance 30 and other foreign matter out of the mass and to cause the smaller-size stones substantially to fill the interstices between the larger-size stones, whereby the resulting floor will be of about the hardness of a solid trap-rock 35 surface.

In testimony whereof, I have hereunto subscribed my name this 13th day of February, 1922.

JOHN MICHAEL TOBIN.